

## UNITED STATES PATENT OFFICE

1,925,645

PROCESS FOR THE MANUFACTURE OF  
FERTILIZERS RICH IN  $P_2O_5$ Vladislav Přistoupil, Aussig on the Elbe,  
CzechoslovakiaNo Drawing. Application March 9, 1931, Serial  
No. 521,398, and in Czechoslovakia March 15,  
1930

5 Claims. (Cl. 71—7)

The present invention relates to a process for the production of fertilizers rich in phosphoric acid from crude phosphates and to the products obtained thereby, it consists in subjecting the 5 crude phosphates at an elevated temperature to the action of phosphorus pentoxide preferably in the form of vapour. Under these conditions the combination of the  $P_2O_5$  with the crude phosphate takes place quickly and completely with the formation of fertilizing substances, which can be easily distributed, having for example a  $P_2O_5$  content up to 60% and over.

This  $P_2O_5$  content can be regulated within fairly wide limits according to the quantities of  $P_2O_5$  employed. Thus for example fertilizers can be manufactured which correspond to calcium pyrophosphate, calcium metaphosphates or mixtures of these, that is to say in which the molecular proportion  $CaO:P_2O_5$  amounts to about 1:½ to 1:1. Fertilizers still richer in phosphoric acid, for example in which the molecular proportion of  $CaO$  to  $P_2O_5$  = 1:2 can also easily be obtained from the crude phosphates.

The fertilizers obtained in this manner are not 25 hygroscopic have good covering power and the solubility of the phosphoric acid is satisfactory for fertilizing purposes. The solubility can be still further increased by effecting a sudden cooling or quenching of the hot, preferably molten, products, care being preferably taken that a large superficial area is produced. The cooling or quenching can be effected for example by pouring the molten product on to cold iron plates 30 or by allowing it to flow into cold water.

One method of carrying the process into effect 35 is to produce the  $P_2O_5$  necessary for the reaction by the combustion of elemental phosphorus, preferably in the form of vapour, and to use the heat 40 of combustion for maintaining the reaction temperature. This method of carrying out the process is particularly advantageous as it enables the phosphorus-containing gases which are formed in the manufacture of phosphorus by reduction 45 of phosphates to be directly utilized. In this case the phosphorus contained in the phosphorus furnace gases is burnt to  $P_2O_5$  in known manner and the heat resulting from this combustion is utilized 50 for maintaining the reaction. The available amount of heat can be still further improved by utilizing the CO content of the phosphorus furnace gases for the development of heat.

## Example

55 Phosphorus-containing gas is burnt with air in

the lower part of a stationary, heat-insulated shaft which is charged with filling material. The gases of combustion containing  $P_2O_5$  spread upwards in the shaft and bring it to the necessary temperature of about 1200° C. Crude phosphate 60 in fine-grained form or in the form of small pieces is continuously fed from above into the shaft. It lies at first on the filling materials. After it has been partly converted by the  $P_2O_5$ , it first becomes tacky and finally liquid and flows over 65 the filling material in the opposite direction to the stream of gas. It thereby takes up further quantities of  $P_2O_5$  and finally collects in the lower part of the furnace where it is run off from time to time and preferably allowed to flow directly 70 into cold water for quenching.

The product obtained can easily be ground to have a size of grain suitable for fertilizing purposes. The phosphoric acid content of the final 75 product, which also depends to some extent on the dimensions of the furnace, can be regulated as desired within wide limits by varying the rate of charging and the speed and composition of the phosphorus-containing gases.

Instead of taking place in the above-described 80 apparatus, the conversion of the crude phosphate may take place for example in an apparatus of the following kind. The molten reaction mass is placed in a heat-insulated, fire-proof container. 85 Into this mass there dips a system of pipes in which the combustion of the gases containing phosphorus vapour is effected. The heat developed is directly transferred to the melt and maintains the necessary temperature. The  $P_2O_5$ -containing 90 combustion gases are driven through the melt in as fine a distribution as possible, whereby the  $P_2O_5$  content is taken up by the mass. The crude phosphate to be converted is continually 95 introduced into the melt and the product of the reaction is run off from time to time in portions and quenched.

## I claim:—

1. Process for the production of fertilizers rich in phosphoric acid from crude phosphates which 100 comprises treating the crude phosphates with phosphorus pentoxide at glowing heat.

2. Process for the production of fertilizers rich in phosphoric acid from crude phosphates which 105 comprises treating the crude phosphates with phosphorus pentoxide at glowing heat and suddenly cooling the products of the reaction.

3. Process for the production of fertilizers rich in phosphoric acid from crude phosphates which 110 comprises treating a crude phosphate with phos-

phorus pentoxide vapour at a temperature of about 1200° C.

4. Process for the production of fertilizers rich in phosphoric acid from crude phosphates which comprises treating the crude phosphate with phosphorus pentoxide at glowing heat until the proportion of combined  $P_2O_5$  is greater than that which would correspond to the production of the metaphosphate.

10

5. Process for the production of fertilizers rich in phosphoric acid from crude phosphates which comprises burning phosphorus to form phosphorus pentoxide treating the crude phosphate with the pentoxide formed at glowing heat, and using the heat of combustion of the phosphorus to maintain the reaction temperature.

VLADISLAV PŘISTOUPIL.

80

85

15

90

20

95

25

100

30

105

35

110

40

115

45

120

50

125

55

130

60

135

65

140

70

145

75

150